

[54] PROCESSING FOR HIGH PERMEABILITY SILICON STEEL COMPRISING COPPER

[75] Inventors: James A. Salsgiver, Sarver; Frank A. Malagari, Freeport, both of Pa.

[73] Assignee: Allegheny Ludlum Industries, Inc., Pittsburgh, Pa.

[22] Filed: May 7, 1973

[21] Appl. No.: 357,974

[52] U.S. Cl. 148/112, 75/123 L, 148/31.55,  
148/111

[51] Int. Cl. H01f 1/04

[58] Field of Search 148/112, 111, 110, 31.55,  
148/113; 75/123 L

[56] References Cited

UNITED STATES PATENTS

|           |         |                      |           |
|-----------|---------|----------------------|-----------|
| 1,919,983 | 7/1933  | Morrill .....        | 148/112   |
| 2,209,686 | 7/1940  | Crafts .....         | 148/31.55 |
| 3,151,005 | 9/1964  | Alworth et al. ....  | 148/111   |
| 3,159,511 | 12/1964 | Taguchi et al. ....  | 148/111   |
| 3,266,955 | 8/1966  | Taguchi et al. ....  | 148/111   |
| 3,287,184 | 11/1966 | Koh .....            | 148/113   |
| 3,632,456 | 1/1972  | Sakakura et al. .... | 148/111   |
| 3,671,337 | 6/1972  | Kumai et al. ....    | 148/112   |

3,764,406 10/1973 Littmann .....

3,770,517 11/1973 Gray et al. ....

148/111  
148/111

OTHER PUBLICATIONS

Saito, A.; Effect of Minor Elements . . . in Silicon Steel; in Nippon Kinzokv, 27, (1963) pp. 191-195.

Kussmann, A., et al.; Gekupferter Stahl Fur . . . Transform.; in Stahl und Eisen, 50, (1930) pp. 1194-1197, (TS 30057).

Primary Examiner—Walter R. Satterfield

Attorney, Agent, or Firm—Vincent G. Gioia; Robert F. Drapkin

[57] ABSTRACT

A process for producing silicon steel having a cube-on-edge orientation and a permeability of at least 1850 (G/O<sub>e</sub>) at 10 oersteds, which includes the steps of: annealing silicon steel prior to a final cold roll at a temperature of from 1400° to 2150°F; cooling the steel from a temperature below 1700°F and above 750°F to a temperature at least as low as 500°F at a rate which is faster than a still air cool and from its maximum annealing temperature to the temperature below 1700°F and above 750°F at a rate which is no faster than a still air cool; and cold rolling the steel at a reduction of at least 80 percent.

18 Claims, No Drawings

**PROCESSING FOR HIGH PERMEABILITY  
SILICON STEEL COMPRISING COPPER**

The present invention relates to a process for producing electromagnetic silicon steel having a cube-on-edge orientation and a permeability of at least 1850 (G/O<sub>e</sub>) at 10 oersteds.

Oriented silicon steels containing 2.60 to 4.0 percent silicon are generally produced by processes which involve hot rolling, a double cold reduction, an anneal before each cold roll and a high temperature texture anneal. Characterizing these steels are permeabilities at 10 oersteds of from about 1790 to 1840 (G/O<sub>e</sub>).

In recent years a number of patents have disclosed silicon steels with permeabilities in excess of 1850 (G/O<sub>e</sub>) at 10 oersteds. Of these, U.S. Pat. Nos. 3,287,183, 3,632,456 and 3,636,579 appear to be the most interesting from a processing standpoint. U.S. Pat. No. 3,287,183 which issued on Nov. 22, 1966 reveals that a steel composed of specific amounts of carbon, silicon, aluminum, sulfur and iron could be processed into a high permeability silicon steel by cold rolling from 5 to 40 percent annealing at a temperature of from 1742° to 2192°F so as to precipitate AlN, cold rolling from 81 to 95 percent, decarburizing and final texture annealing. More recently, similar processing for similar alloys was disclosed in U.S. Pat. Nos. 3,632,456 and 3,636,579, which respectively issued on Jan. 4, 1972, and Jan. 25, 1972. Each of these patents refer to cooling rates following the anneal in which AlN is precipitated. U.S. Pat. No. 3,632,456 anneals a hot rolled band at a temperature of from 1382° to 2192°F, depending upon its silicon content, rapidly cools the annealed band and then proceeds to subject it to at least two cold rollings. U.S. Pat. No. 3,636,579 anneals steel containing 2.5 to 4 percent silicon at a temperature of from 1742° to 2192°F, quenches it from said temperature to a temperature at least as low as 752°F and then cold rolls it.

Described herein is another, and improved method for producing silicon steel having a cube-on-edge orientation and a permeability of at least 1850 (G/O<sub>e</sub>) at 10 oersted from steel of a particular chemistry. The method includes the steps of: annealing silicon steel prior to a final cold roll at a temperature of from 1400° to 2150°F; cooling the steel from a temperature below 1700°F and above 750°F to a temperature at least as low as 500°F at a rate which is faster than a still air cool and from its maximum annealing temperature to the temperature below 1700°F and above 750°F at a rate which is no faster than a still air cool; and cold rolling the steel at a reduction of at least 80 percent. It differs from and is contradictory to the methods of heretofore referred to U.S. Pat. Nos. 3,287,183, 3,632,456 and 3,636,579 in that: U.S. Pat. No. 3,287,183 does not relate to cooling rates; U.S. Pat. No. 3,632,456 calls for an anneal and two cold rollings subsequent to the anneal aimed at precipitating AlN and the rapid cool which occurs thereafter; and both U.S. Pat. Nos. 3,632,456 and 3,636,579 refer to rapid cools from a temperature in excess of 1742°F, for steels containing at least 2.5% Si. Moreover, the chemistry of the steel being processed in accordance with the present invention differs from that being processed in said heretofore referred to patents.

It is accordingly an object of the present invention to provide a process for producing electromagnetic sili-

con steel having a cube-on-edge orientation and a permeability of at least 1850 (G/O<sub>e</sub>) at 10 oersteds.

The present invention provides a method for producing silicon steel having a cube-on-edge orientation and a permeability of at least 1850 (G/O<sub>e</sub>), and preferably at least 1900 (G/O<sub>e</sub>), at 10 oersteds. Involved therein are the steps of: preparing a melt of silicon steel having, by weight, up to 0.07% carbon, from 2.60 to 4.0% silicon, from 0.03% to 0.24% manganese, from 0.01 to 0.07% sulfur, from 0.015 to 0.04% aluminum, up to 0.02% nitrogen, and from 0.1 to 0.5% copper; casting the steel; hot rolling the steel into a hot rolled band; subjecting the steel to at least one cold rolling and generally two; subjecting the steel to a final annealing prior to the final cold rolling; decarburizing the steel; and final texture annealing the steel. Also included, and significantly so, are the specific steps of: carrying out the final anneal prior to the final cold rolling at a temperature of from 1400° to 2150°F for a period of from 15 seconds to 2 hours; cooling the steel from a temperature below 1700°F and above 750°F to a temperature at least as low as 500°F at a rate which is faster than a still air cool and from its maximum annealing temperature to the temperature below 1700°F and above 750°F at a rate which is no faster than a still air cool; and cold rolling the cooled steel at a reduction of at least 80 percent. Preferred conditions include annealing at a temperature of from 1800° to 2125°F, cooling at a rate faster than a still air cool from a temperature below 1600°F and above 1200°F, and cold rolling at a reduction of at least 85 percent. No critically is placed upon the means for obtaining a cooling rate faster than a still air cool. Illustrative means are gaseous streams and liquid quenching mediums. For purposes of definition, still air cools include those wherein the steel is cooled in a static atmosphere as well as those wherein there is relative motion between the atmosphere and the steel, as in a continuous processing line, so long as there is no deliberate intention to cause the motion for cooling purposes. Moreover, for purposes of definition, all gaseous atmospheres are considered to have the same cooling effect as air. Hence, all cools are considered to be at a rate no faster than a still air cool unless a liquid quenching medium or forced gaseous atmosphere is employed, and a forced gaseous atmosphere is one in which motion is deliberately imparted to the atmosphere for cooling purposes.

Melting, casting, hot rolling, cold rolling, decarburizing and final texture annealing do not involve any novel procedure, as far as techniques are concerned, and with regard to them, the invention encompasses all applicable steelmaking procedures. As to the cold rolling, it should, however, be pointed out that several roll passes can constitute a single cold rolling operation, and that plural cold rolling operations exist only when cold rolling passes are separated by an anneal.

The steel melt must include silicon, aluminum, manganese, sulfur and copper. Silicon is necessary as it increases the steel's resistivity, decreases its magnetostriction, decreases its magnetocrystalline anisotropy and hence decreases its core loss. Aluminum, manganese and sulfur are necessary as they form inhibitors which are essential to controlling the steel's orientation and its properties which are dependent thereon. More specifically, aluminum combines with nitrogen, in the steel or from the atmosphere to form aluminum nitride, and manganese combines with sulfur to form manga-

nese sulfide and/or manganese copper sulfide; and these compounds act so as to inhibit normal grain growth during the final texture anneal, while at the same time, aiding in the development of secondary recrystallized grains having the desired cube-on-edge orientation. Copper, in addition to possibly forming manganese copper sulfide, is believed to be beneficial in that it is hypothesized that copper can lower the annealing temperature, lower the temperature from which the rapid cool can occur, improve rollability, simplify melting and relax annealing atmosphere requirements. Alloys with more than 0.15 percent copper have been successfully annealed prior to the final cold rolling at temperatures of from 1400° to 1700°F.

A steel in which the process of the present invention is particularly adaptable to consist essentially of, by weight, from 0.02 to 0.07% carbon, from 2.60 to 3.5% silicon, a manganese equivalent of from 0.05 to 0.24% as expressed by an equivalency equation of  $\% \text{Mn} + (0.1 \text{ to } 0.25) \times \% \text{Cu}$ , from 0.01 to 0.5% sulfur, from 0.015 to 0.04% aluminum, from 0.0030 to 0.0090% nitrogen, from 0.1 to 0.3% copper, balance iron and residuals; and wherein the ratio of manganese equivalent to sulfur is in the range of from 2.0 to 4.75. The steel has its chemistry balanced so as to produce a highly beneficial structure when processed according to the present invention.

Although we are not sure why the annealing and cooling of the present invention is so beneficial, we hypothesize: that the anneal conditions the steel for cold rolling and provides an operation during which inhibitors can form; and that the slow cool to a temperature below 1700°F and /or the use of annealing temperatures in the lower part of the annealing temperature range, increase the uniformity in which the inhibitors are distributed, as essentially only ferrite phase is present in the steel at temperatures below 1700°F, contrasted to the presence of austenite and ferrite phases and different solubilities for the inhibiting elements in each phase at somewhat higher temperatures. As discussed above, the primary inhibitors are aluminum nitride and manganese sulfide and/or manganese copper sulfide. No criticality is placed upon the particular annealing atmosphere. Illustrative atmospheres therefore include nitrogen; reducing gases such as hydrogen; inert gases such as argon; air; and mixtures thereof.

The following examples are illustrative of several aspects of the invention.

#### EXAMPLE I

Twelve samples (Samples 1 - 12) of silicon steel were cast and processed into silicon steel having a cube-on-edge orientation from two heats (Heats A and B) of BOF silicon steel. The chemistry of the heats, that is Heats A and B, appears hereinbelow in Table I.

TABLE I

| COMPOSITION (Wt. %) |       |      |       |      |       |      |        |      |  |
|---------------------|-------|------|-------|------|-------|------|--------|------|--|
| Heat                | C     | Mn   | S     | Si   | Al    | Cu   | N      | Fe   |  |
| A                   | 0.051 | 0.13 | 0.042 | 2.97 | 0.031 | 0.24 | 0.0037 | Bal. |  |
| B                   | 0.038 | 0.10 | 0.03  | 2.94 | 0.027 | 0.23 | 0.0047 | Bal. |  |

Processing for the twelve samples involved soaking at an elevated temperature for several hours, blooming, hot rolling to a gage of approximately 130 mils, normal-

izing for 2 minutes at 1650°F in air, cold rolling to a gage of approximately 88 mils, annealing a 2000°F for 5 minutes in nitrogen, cooling by one of three cooling methods (Cooling Methods, I, II or III), cold rolling to final gage of approximately 12 mils, decarburizing for 2 minutes at 1475°F in a mixture of nitrogen and wet hydrogen, and final annealing for 8 hours in hydrogen at a maximum temperature of 2150°F. Cooling Method I was applied to samples 1, 4, 7 and 10, and is one in which the samples are cooled in a welded box. It is a cool which is slower than an air cool. Samples 1, 4, 7 and 10 took approximately 50 minutes to cool to 750°F. Cooling Method II was applied to samples 2, 5, 8 and 11, and is one in which the samples are furnace cooled to 1600°F and air cooled therefrom. Furnace cooling to 1600°F took approximately 20 minutes. Cooling from 1740° to 1600°F took approximately 8 minutes. Cooling Method III was applied to samples 3, 6, 9 and 12, and is the same as Cooling Method II with the exception that the samples were brine quenched at 1600°F.

Samples 1 - 12 were tested for permeability and core loss. The results of the tests appear hereinbelow in Table II. Results have been broken up into four groups so that only samples from the same heat and coil are directly compared. Samples 1, 2 and 3 are from the same heat and coil and form one group, as do samples 4, 5 and 6, samples 7, 8 and 9, and samples 10, 11 and 12.

TABLE II

| Sample | Heat | Cooling Method | Permeability (at 10 O <sub>e</sub> ) | Core Loss (WPP at 17 KB) |
|--------|------|----------------|--------------------------------------|--------------------------|
| 1      | A    | I.             | 1848                                 | 0.879                    |
| 2      | A    | II.            | 1893                                 | 0.793                    |
| 3      | A    | III.           | 1928                                 | 0.715                    |
| 4      | A    | I.             | 1846                                 | 0.908                    |
| 5      | A    | II.            | 1910                                 | 0.738                    |
| 6      | A    | III.           | 1931                                 | 0.718                    |
| 7      | B    | I.             | 1830                                 | 0.887                    |
| 8      | B    | II.            | 1878                                 | 0.835                    |
| 9      | B    | III.           | 1908                                 | 0.731                    |
| 10     | B    | I.             | 1831                                 | 0.942                    |
| 11     | B    | II.            | 1903                                 | 0.769                    |
| 12     | B    | III.           | 1914                                 | 0.728                    |

From Table II, it is clear that the processing of the present invention is highly beneficial to the properties of silicon steel having a cube-on-edge orientation. Samples 3, 6, 9 and 12 were annealed in nitrogen for 5 minutes at 2000°F, cooled to 1600°F at a rate slower than a still air cool and cooled from 1600°F to a temperature below 500°F at a rate faster than a still air cool; and all had permeabilities in excess of 1900 (G/O<sub>e</sub>) at 10 O<sub>e</sub>. On the other hand, samples 1, 4, 7 and 10 which were annealed as were samples 3, 6, 9 and 12, but not cooled from a temperature in excess of 750°F at a rate faster

than a still air cool, all had permeabilities less than 1850 (G/O<sub>e</sub>) at 10 O<sub>e</sub>. Having permeabilities between the values for samples 3, 6, 9 and 12, and samples 1, 4,

7 and 10 were samples 2, 5, 8 and 11. These samples were annealed as were the other samples, and cooled to 1600°F as were samples 3, 6, 9 and 12, but unlike samples 2, 6, 9 and 12 they were not cooled from 1600°F at a rate faster than a still air cool. This permeabilities were high but not as high as those of samples 3, 6, 9 and 12, the samples processed in accordance with the present invention. Moreover, samples 3, 6, 9 and 12 had lower core losses than did samples 2, 5, 8 and 11, and samples 2, 5, 8 and 11 had lower core losses than did samples 1, 4, 7 and 10. Of course, all comparisons are made for the respective groups.

#### EXAMPLE II

Three additional samples (Samples 14 – 16) of silicon steel were cast and processed into silicon steel having a cube-on-edge orientation from a third heat (Heat C) of BOF silicon steel. The chemistry of the heat, that is Heat C, appears hereinbelow in Table III.

TABLE III

| COMPOSITION (Wt. %) |       |       |       |      |       |      |        |      |
|---------------------|-------|-------|-------|------|-------|------|--------|------|
| Heat                | C     | Mn    | S     | Si   | Al    | Cu   | N      | Fe   |
| C                   | 0.049 | 0.094 | 0.032 | 2.91 | 0.036 | 0.22 | 0.0046 | Bal. |

Processing for the three samples involved soaking at an elevated temperature for several hours, blooming, hot rolling to a gage of approximately 92 mils, annealing at 1475°F for 1 hour in nitrogen, cooling by one of three methods, cold rolling a final gage of approximately 13 mils, decarburizing for 2 minutes at 1475°F in a mixture of nitrogen and wet hydrogen, and final annealing for 8 hours in hydrogen at a maximum temperature of 2150°F. The three cooling methods were a furnace cool, an air cool and a brine quench. Sample 14 was furnace cooled, sample 15 was air cooled, and the brine quench was applied to sample 16.

Samples 14 – 16 were tested for permeability and core loss. The results of the tests appear hereinbelow in Table IV.

TABLE IV

| Sample | Heat | Cooling      | Permeability<br>(at 10 O <sub>e</sub> ) | Core Loss<br>(WPP at 17 KB) |
|--------|------|--------------|-----------------------------------------|-----------------------------|
| 14     | C    | Furnace      | 1651                                    | 1.27                        |
| 15     | C    | Air          | 1860                                    | 0.785                       |
| 16     | C    | Brine Quench | 1902                                    | 0.708                       |

From Table IV, it is clear that the processing of the present invention is highly beneficial to the properties of silicon steel having a cube-on-edge orientation, and from Tables II and IV, it is clear that this processing is beneficial whether there is only one cold rolling as in Example II or at least two cold rollings as in Example I. Sample 16 was annealed in nitrogen for 1 hour at 1475°F and cooled therefrom to a temperature below 500°F at a rate faster than a still air cool; and had a permeability in excess of 1900 (G/O<sub>e</sub>) at 10 O<sub>e</sub>. On the other hand, sample 14 which was annealed as was sample 16, but not cooled from a temperature in excess of 750°F at a rate faster than a still air cooled from a temperature in excess of 750°F at a rate faster than a still air cool, had a permeability considerably below 1850 (G/O<sub>e</sub>) at 10 O<sub>e</sub>. Having a permeability between the

values for samples 16 and 14 was sample 15. It was annealed as were samples 16 and 14, but unlike sample 16 was not cooled from 1475°F at a rate faster than a still air cool. The permeability for this sample was high but not as high as that for sample 16, the same processed in accordance with the present invention. Moreover, sample 16 had a lower core loss than did sample 15, and sample 15 had a lower core loss than did sample 14.

It will be apparent to those skilled in the art that the novel principles of the invention disclosed herein in connection with specific examples thereof will suggest various other modifications and applications of the same. It is accordingly desired that in construing the breadth of the appended claims they shall not be limited to the specific examples of the invention described herein.

We claim:

1. In a process for producing electromagnetic silicon

steel having a cube-on-edge orientation and a permeability of at least 1850 (G/O<sub>e</sub>) at 10 oersteds, which process includes the steps of: preparing a melt of silicon steel; casting said steel; hot rolling said steel into a hot rolled band; subjecting said steel to at least one cold rolling; subjecting said steel to a final annealing prior to the final cold rolling; decarburizing said steel; and final texture annealing said steel; the improvement comprising the steps of carrying out said final anneal prior to the final cold rolling at a temperature of from 1400° to 2150°F for a period of from 15 seconds to 2 hours; cooling said steel from a temperature below 1700°F and above 750°F to a temperature at least as low as 500°F with a liquid quenching medium or gaseous stream and from its maximum annealing temperature to said temperature below 1700°F and above 750°F at a rate which is no faster than one wherein the steel is cooled in a static atmosphere or in a continuous processing line where there is some relative motion between the atmosphere and the steel, although the only deliberate motion is that imparted to the steel; and cold rolling the cooled steel at a reduction of at least 80 percent; said melt consisting essentially of, by weight, up to 0.07% carbon, from 2.60 to 4.0% silicon, from 0.03 to 0.24% manganese, from 0.01 to 0.07% sulfur, from 0.015 to 0.04% aluminum, up to 0.02% nitrogen, from 0.1 to 0.5% and the balance iron.

2. An improvement according to claim 1, wherein said steel is cooled from a temperature below 1600°F and above 1200°F to a temperature at least as low as 500°F at a rate which is faster than a still air cool and from its maximum annealing temperature to said temperature below 1600°F and above 1200°F at a rate which is no faster than a still air cool.

3. An improvement according to claim 1, wherein said final anneal prior to the final cold rolling is at a temperature of from 1800° to 2125°F.

4. An improvement according to claim 3, wherein said steel is cooled from a temperature below 1600°F

and above 1200°F to a temperature at least as low as 500°F at a rate which is faster than a still air cool and from its maximum annealing temperature to said temperature below 1600°F and above 1200°F at a rate which is no faster than a still air cool.

5. An improvement according to claim 1 wherein said steel is cooled to a temperature at least as low as 500°F from a temperature below 1700°F and above 750°F with a gaseous stream.

6. An improvement according to claim 1 wherein said steel is cooled to a temperature at least as low as 500°F from a temperature below 1700°F and above 750°F with a liquid quenching medium.

7. An improvement according to claim 1 wherein said steel is air cooled to said temperature below 1700°F and above 750°F.

8. An improvement according to claim 3 wherein said steel is cooled to a temperature at least as low as 500°F from a temperature below 1700°F and above 750°F with a gaseous stream.

9. An improvement according to claim 3 wherein said steel is cooled to a temperature at least as low as 500°F from a temperature below 1700°F and above 750°F with a liquid quenching medium.

10. An improvement according to claim 3 wherein said steel is air cooled to said temperature below 1700°F and above 750°F.

11. An improvement according to claim 1, wherein said final anneal prior to the final cold rolling is carried out subsequent to an initial cold rolling.

12. An improvement according to claim 1, wherein

said steel consists essentially of, by weight, from 0.02 to 0.07% carbon, from 2.60 to 3.5% silicon, a manganese equivalent of from 0.05 to 0.24% as expressed by an equivalency equation of % Mn + (0.1 to 0.25) × %

5 Cu, from 0.01 to 0.05% sulfur, from 0.015 to 0.04% aluminum, from 0.0030 to 0.0090% nitrogen, from 0.1 to 0.3% copper, balance iron and residuals; and wherein the ratio of manganese equivalent to sulfur is in the range of from 2.0 to 4.75.

10 13. An improvement according to claim 1, wherein the cooled steel is cold rolled at a reduction of at least 85 percent.

14. An improvement according to claim 4, wherein the cooled steel is cold rolled at a reduction of at least 85 percent.

15 15. An improvement according to claim 1 wherein said final anneal prior to the final cold rolling is applied to a hot rolled band.

20 16. An improvement according to claim 1 wherein said steel has at least 0.15% Cu and wherein said final anneal prior to the final cold rolling is at a temperature of from 1400° to 1700°F.

17. An improvement according to claim 16 wherein said steel is cooled to a temperature at least as low as 500°F from a temperature above 750°F with a gaseous stream.

25 18. An improvement according to claim 16 wherein said steel is cooled to a temperature at least as low as 500°F from a temperature above 750°F with a liquid quenching medium.

\* \* \* \* \*

35

40

45

50

55

60

65